

# United States Patent Office

2,970,907

Patented Feb. 7, 1961

1

2,970,907

## PHYSICAL PROPERTIES OF PHOTOGRAPHIC PAPERS

Joseph Sottysiak, Binghamton, and Benjamin R. Harriman, Rochester, N.Y., assignors to General Aniline & Film Corporation, New York, N.Y., a corporation of Delaware

No Drawing. Filed Apr. 20, 1956, Ser. No. 579,433

8 Claims. (Cl. 96—85)

The present invention relates to protective layers for photographic silver halide emulsion layers, particularly anti-abrasion protective layers especially for photographic papers.

Photographic papers, usually the so-called glossy types, are generally provided with a protective overcoating comprising gelatin. Such papers, with or without such overcoating, after being exposed and processed, are squeegeed and dried against a very highly polished metal surface in order to produce highly glossed prints by ferrotyping. The gelatins which are used in the emulsions or protective layers are generally selected for excellence in certain properties but often manifest very poor ferrotyping characteristics. Thus, it is often experienced that the processing solutions or the wash water contain salts which impair ferrotyping. As a consequence, the ferrotyped prints frequently exhibit a low gloss caused by these and other factors. Close examination establishes the low gloss and ferrotyping imperfections to be attributable to defects known as pits, "edge lift" and "oyster shells."

"Edge lift," as is known in the art, means the dullness at the edges of the prints caused by insufficient length of contact between the edges of the print and the polished metal surface. "Oyster shells," on the other hand, refer to the concentric circles in prints occasioned by improper drying.

Bower et al., in their U.S. Patent 2,633,423, suggested that these defects might be cured by substituting for the conventional gelatin overcoat a layer of a hydantoin-formaldehyde resin. It is claimed that such resin coatings not only impart anti-abrasion properties to the gelatin-silver halide layer but also give smoother surfaces, less warping and a better over-all appearance to the finished product, particularly photographic paper.

It has also been suggested that poor ferrotyping can be obviated or suppressed by careful operation in processing. It has been found, however, that this procedure materially slows up the operation while requiring the use of additional chemicals and techniques.

It has now been discovered that the problems mentioned with respect to ferrotyping, particularly of photographic paper, can be overcome by overcoating the silver halide emulsion layer with an anti-abrasion gelatin coating containing an anionic or non-ionic surface active agent alone or preferably with beeswax.

It is, accordingly, an object of the present invention to provide an anti-abrasion layer on photographic paper, permitting ferrotyping with high gloss when the paper is contacted with a polished metal surface.

A further object of the invention is to build into the photographic paper protection against ferrotyping defects.

A still further object of the invention is to enable the ferrotyping of prints while ensuring that the resulting gloss is free from pitting, "edge lift" and "oyster shells."

Other and further important objects will appear as the description proceeds.

2

As previously stated, our invention is predicated upon the incorporation in a gelatin protective layer of a surface active agent which is chosen for its ability to orient itself on the surface of the photographic material in such a way as to provide the desired ferrotyping characteristics. Surface active agents which meet these prerequisites are any of the anionic or non-ionic surface active agents. Surface active agents of the anionic and non-ionic class are well known in industry and are available on the open market. Examples of the anionics which we have found to be particularly suitable are sodium tetradecyl sulfate, sodium octyl phosphate, the sodium salt of aromatic sulfonic acids such as the sodium salt of butyl naphthalene sulfonic acid, the sodium salt of keryl benzene sulfonic acid (the product resulting from the condensation of chlorinated kerosene with benzene followed by sulfonation), monodiethylaminoethyldecenyl succinate, U.S. Patent 2,805,948, and the like. Examples of non-ionic surfactants are diglycol laurate, the condensation products of compounds containing a reactive hydrogen atom with ethylene oxide such as the products described in U.S. Patent 1,970,578, specifically, 2,6,8-trimethyl nonanol-4 with 12 mols of ethylene oxide, diethyl phenol with 20 mols of ethylene oxide and the like and the condensation products of long chain fatty acids with proteins such as those described in U.S. Patent 2,015,912. Best results were secured with the succinic acid derivative and we, accordingly, prefer the use of this compound.

30 The effective concentration of the surface active agent in the gelatin ranges from 2.5 to 125 grams per kilo of gelatin and preferably from 5 to 10 grams per kilo.

It has been ascertained that, while the ferrotyping properties are materially augmented by the use of the surfactant alone, such properties are even further improved if there be incorporated into the gelatin-surfactant mixture, an addition of a beeswax emulsion. The beeswax should be of purest possible grade to ensure freedom from photographic contamination, on the one hand, and uniformity of ferrotyping, on the other hand. Purified white disc beeswax is suitable such as that supplied by the Norda Essential Oil and Chemical Company or the Frank B. Ross Company, Inc.

The wax is used in an amount of 50 to 400 grams per kilogram of gelatin in the protective overcoating. The quantities of the surface active agent used in combination with the wax and gelatin are the same as specified above, to wit, 2.5 to 125 grams per kilo with preference for the lower range.

50 We have found that the gelatin overcoating, for reasons which we have been unable to ascertain, gives optimum results when there is used with the aforesaid components a stabilizer for silver halides, for example, those described in U.S. Patents 2,440,110; 2,440,206; 2,385,762; and 2,394,198. The quantity of stabilizer would be within the range stated in said patents.

55 The invention is further illustrated by the following examples, it being understood, however, that the invention is not restricted thereto.

60

### Example I

A 2% gelatin solution was prepared by dissolving one kilogram of gelatin in distilled water. This gelatin solution was heated to 30° C. and to it were added 300 mls. of 10% chrome alum solution, a silver halide stabilizer (of the type and in the quantity mentioned in U.S. Patent 2,440,110) and 7.5 grams of monodiethylaminoethyldecenyl succinate. In a separate container, 125 grams of beeswax and 6.3 mls. of triethanolamine were heated to 65° C. and poured into 1250 mls. of water at 65° C. The resulting beeswax emulsion was cooled to 30° C. and an additional 1250 mls. of distilled water were

added. The 2500 mls. of wax emulsion were added to the gelatin solution with stirring at 30° C. and the solution was coated at this temperature over a wet chilled gelatino-silver halide layer on a paper support. This protective layer dried down to a thickness of about 1 5 micron.

This photographic paper was compared with a similar paper which differed only in that the protective layer was made from a 2% gelatin solution to which had been added chrome alum, the stabilizer and 100 grams of saponin. Both papers were exposed, processed in the 10 normal manner and then, after washing, placed emulsion side down upon a cold polished metal surface for simultaneous drying and ferrotyping. The paper with the protective layer containing the beeswax and succinic acid derivative had much better resistance to surface defects such as pitting and "edge lift."

#### Example II

The procedure is the same as in Example I, excepting 20 that the beeswax emulsion is omitted. The paper with the protective layer containing the monodiaminoethyl-dodeceny succinate had far better resistance toward physical defects than a similar paper in which the protective layer is free from such surfactant.

#### Example III

The procedure is the same as in Example I, excepting 30 that the paper was ferrotyped upon a hot polished metal plate. The improvements noted in Example I were also observed in this instance.

#### Example IV

The procedure is the same as in Example II, excepting 35 that the paper was ferrotyped upon a hot polished metal surface. In this case, resistance towards physical defects was again observed.

Modification of the invention will occur to persons skilled in the art and we, therefore, do not intend to be limited in the patent granted except as necessitated by 40 the appended claims.

We claim:

1. Light-sensitive photographic paper having excellent 45 ferrotyping characteristics comprising a paper base coated with a gelatino silver halide emulsion which, in turn, is overcoated with a thin layer of gelatin having dispersed

therethrough as the sole surfactant a surface active agent selected from the class consisting of monodiethylaminoethyl-dodeceny succinate, the condensation product of 2,6,8-trimethylnonanol-4 with ethylene oxide and the condensation product of diethylphenol with ethylene oxide.

2. The article as defined in claim 1, wherein the gelatin overcoat contains beeswax in an amount ranging from 50 to 400 grams per kilo of gelatin.

3. Light-sensitive photographic paper having excellent ferrotyping characteristics, comprising a base coated with a gelatino silver halide emulsion which is, in turn, overcoated with a thin layer of gelatin having dispersed therethrough as the sole surfactant a surface active agent selected from the group consisting of monodiethylaminoethyl-dodeceny succinate, the condensation product of 2,6,8-trimethylnonanol-4 with 12 mols of ethylene oxide and the condensation product of diethylphenol with 20 mols of ethylene oxide; a stabilizing amount of a stabilizer for silver halides, and beeswax.

4. The article as defined in claim 1, wherein the surfactant is present in an amount ranging from 2.5 to 125 grams per kilo of gelatin.

5. The article as defined in claim 1, wherein the gelatin overcoat contains a stabilizing quantity of a silver halide stabilizer.

6. The article as defined in claim 1, wherein the surface active agent is monodiethylaminoethyl-dodeceny succinate.

7. The article defined in claim 2, wherein the surface active agent is monodiethylaminoethyl-dodeceny succinate.

8. The article as defined in claim 3, wherein the surface active agent is monodiethylaminoethyl-dodeceny succinate.

#### References Cited in the file of this patent

##### UNITED STATES PATENTS

|           |               |                |
|-----------|---------------|----------------|
| 2,368,287 | Chilton       | Jan. 30, 1945  |
| 2,440,110 | Mueller       | Apr. 20, 1948  |
| 2,465,149 | Dersch et al. | Mar. 22, 1949  |
| 2,600,831 | Baldsiefen    | June 17, 1952  |
| 2,719,087 | Knox et al.   | Sept. 27, 1955 |
| 2,726,955 | Parnell       | Dec. 13, 1955  |

##### FOREIGN PATENTS

|         |               |              |
|---------|---------------|--------------|
| 418,976 | Great Britain | Nov. 5, 1934 |
|---------|---------------|--------------|